

## UNITED STATES PATENT OFFICE

WARREN K. LEWIS, OF NEWTON, MASSACHUSETTS, ASSIGNOR TO STANDARD OIL DEVELOPMENT COMPANY, A CORPORATION OF DELAWARE

## PROTECTIVE COATING

No Drawing.

Application filed April 1, 1929. Serial No. 351,829.

The present invention relates to protective coverings and more specifically to a protective coating for metals exposed to the action of petroleum or petroleum vapors. My invention will be fully understood from the following description.

Oil tanks used for the storage of crude and partially refined oils are subject to extremely severe conditions of internal corrosion, particularly when used for storage of high sulphur-containing oil such as are produced in West Texas fields and in other localities. Tank roofs, the upper plates, and the internal braces are quickly corroded, presumably by the combined effects of the oil or oil vapor, moisture, and the sulphur-containing impurities in the oil.

I have invented a new type of protective coating which is cheap, resistant, and easily applied and by its use the life of tank roofs and other metal parts may be greatly extended. The coating is made up essentially of two parts, a first layer which is substantially impermeable to moisture, but which is more or less rapidly effected by oil or oil vapors and a second coating applied over the first which is substantially impermeable and unaffected by oil, oil vapor or its corrosive impurities, and is substantially insoluble in water.

The metal surface to be covered is first preferably cleaned by scraping in the usual manner and removing rust spots. The first coating is then applied and is preferably one or more coats of a good oil paint, such as a lead paint or zinc paint. Mixed base paints may also be used and particularly those containing fine divided metals such as aluminum or bronze.

After the paint has dried thoroughly the second coating is applied. This comprises a glue composition which contains a suitable fixing agent adapted to render the glue water insoluble. A good quality hide glue is preferable because of its cost and durability, but bone glues or fish glues may be used as well. A small percentage, say  $\frac{1}{2}$  to 2% of para-aldehyde is added to the glue solution as the fixing agent, although formaldehyde, tannic acid, potassium bichromate or the like may

be used. It may be preferable to apply the glue and later treat the surface with the fixing agent either in aqueous solution or as a gas in the use of formaldehyde. In any case, it is generally advisable to add 20 to 50% of glycerine in the weight of the dry glue, and to also add a small quantity, say  $\frac{1}{4}$  to  $\frac{1}{2}\%$  of oxalic acid to prevent too rapid hardening.

The glue is made up in a thick solution with water which may be heated and it is diluted to the proper consistency for brushing or spraying. For brushing two pounds of dry glue per gallon of water has proved satisfactory altho it may be varied considerably. For spraying generally more dilute solutions are preferable.

Instead of applying the glue as a solution directly to the painted metal, paper or other suitable absorbent fabric, preferably of a vegetable nature may be impregnated with the solution and after it has dried the fabric may be applied to the painted metal either by glue or other adhesives such as rubber cement, or bitumen or by suitable mechanical means. It may be advantageous in some cases to apply a glue solution over the impregnated fabric to fix the glue as heretofore specified.

While good quality paint is preferable for the first coating cellulose esters or ethers such as nitro-cellulose or cellulose acetate may be used in an appropriate solvent. Gums, resins, bitumen and the like may also be added to the paint to increase its effectiveness or asphalt or bitumen may be used instead of a drying oil paint.

My invention is not to be limited by any theory of the manner in which my improved coating is applied or operates, nor by any illustrative example of the particular composition of either of the two coatings which are given merely for purposes of illustration, but only by the following claims in which I wish to claim all novelty inherent in the invention.

I claim:

1. The method of protecting oil containers used for the storage of crude and partially refined oil from deterioration, which comprises coating the body with paint substan-

tially impervious to moisture, and applying a surface coating of animal glue to the coating of paint.

2. The method of protecting oil containers used for the storage of crude and partially refined oil from deterioration, which comprises coating the body with paint substantially impervious to moisture, applying a surface coating of animal glue to the coating of paint, and treating the surface coating with a fixing agent adapted to chemically render the glue insoluble in water.

3. An article of manufacture impervious to corrosive action of oil, oil vapor or its corrosive impurities, comprising a metallic body portion, a layer of water proof paint, and a surface coating of animal glue.

4. An article of manufacture impervious to corrosive action of oil, oil vapor or its corrosive impurities, comprising a metallic body portion, a layer of water proof paint, and a surface coating of animal glue insoluble in water.

5. The method of protecting the internal structure of oil containers used for the storage of crude and partially refined oil from corrosives, which comprises coating the structure with paint substantially impervious to moisture, applying a surface coating of animal glue to the coating of paint, and treating the surface coating with a fixing agent adapted to chemically render the glue insoluble in water.

**WARREN K. LEWIS.**